# EUROPEAN PATENT SPECIFICATION

(11) **EP 0 503 081 B1**
(45) Date of publication and mention of the grant of the patent: **12.06.1996**
(21) Application number: 91916787.4
(22) Date of filing: 27.09.1991
(51) Int. Cl.: H01F 27/245, H01F 3/02, H01F 1/147, H01F 3/04, H01F 27/25, H01F 1/153

(54) **MAGNETIC CORE**
MAGNETKERN
NOYAU MAGNETIQUE

(30) Priority: 28.09.1990 JP 256966/90
(43) Date of publication of application: 16.09.1992
(73) Proprietor: KABUSHIKI KAISHA TOSHIBA, Kawasaki-shi, Kanagawa-ken 210 (JP)
(72) Inventor: OKAMURA, Masami, Yokohama-shi, Kanagawa ken (JP); KUSAKA, Takao, Yokohama-shi, Kanagawa ken (JP)
(74) Representative: Lehn, Werner, Dipl.-Ing.
(86) International application number: JP9101294
(87) International publication number: WO9206480

(56) References cited:
- EP-A- 0 086 485
- DE-A- 2 103 523
- DE-A- 4 002 999
- JP-A- 1 290 746
- JP-A- 2 077 555
- JP-A- 3 124 008
- JP-A-54 082 027
- PATENT ABSTRACTS OF JAPAN vol. 13, no. 513 (E-847)16 November 1989

## Description

### TECHNICAL FIELD

The present invention relates to a magnetic core used in apparatuses such as pulse generators and transformers, and more particularly, to a magnetic core used in a large electric power such as a magnetic core for a high output pulse.

### BACKGROUND ART

Magnetic pulse compression circuits adapted for generating a pulse having a high output and a short pulse duration have been used in pulse power source apparatuses used in lasers and particle accelerators. The magnetic pulse compression circuits compress a current pulse duration utilizing a saturation characteristic of a saturable magnetic core when the charge of a capacitor is shifted to a capacitor of a next stage.

An induction magnetic core of a linear accelerator essentially operates as a 1:1 transformer and accelerates a charged particle beam which passes through the central portion of the magnetic core by means of a voltage generated in a secondary gap.

Heretofore, as these magnetic cores for high output pulse there have been used magnetic cores wherein magnetic material ribbons such as iron-base amorphous alloy ribbons or cobalt-base amorphous alloy ribbons having characteristics such as high saturation magnetic flux density, a high squareness ratio of a magnetization curve and a low core loss and electrical insulating materials composed of a polymeric film such as a polyester film or polyimide film are alternately wound.

In such magnetic cores, an insulating property between magnetic material ribbons is important because the magnetic cores are used in high output pulse applications. Therefore in the prior art in order to ensure layer insulation between magnetic material ribbon edges, the electrical insulating materials and the magnetic material ribbons have been set so that the width of the electrical insulating materials is wider than the width of the magnetic material ribbons.

However, we have now found that the following problems pose in the magnetic cores wherein the width of the electrical insulating materials is wider than the width of the magnetic material ribbons in order to ensure layer insulation between magnetic material ribbons as described above.

That is, as shown in FIG. 2 which is a schematic view of a cross-section of the prior art magnetic core, the edges of an electrical insulating material 2 projects from the edges of a magnetic material ribbon 1. Further, in general the electrical insulating material 2 has a low heat conduction property and therefore the space between the projected portions of the electrical insulating material 2 can be a thermal insulation layer 3. Accordingly, an effect of cooling on the heat generation of magnetic cores in use, in other words, the heat generation of magnetic material ribbons is reduced and thus the temperature of the magnetic cores can rise. In general, while the magnetic cores are cooled by coolant such as air, insulating oils, and fluorine-containing inert liquids, the temperature rise of the magnetic cores can result in the reduction of the magnetic flux of the magnetic cores and the acceleration of secular change of characteristics and there is inevitably occurred a problem that specific functions are not obtained.

From JP-A-1 290 746 (A) a soft magnetic alloy having high saturation magnetic flux density is known.

From DE 40 02 999 A1 a lapped magnetic core consisting of a soft magnetic material and a heat resistance isolation layer is known.

An object of the present invention is to solve the problems described above and provide a magnetic core having an excellent cooling characteristic.

### DISCLOSURE OF INVENTION

This object is solved as defined in claim 1.

A magnetic core of the present invention is a magnetic core obtainable by laminating or winding a magnetic material ribbon and an electrical insulating material wherein it has the relationship of 0.5a ≤ b < a in which the width of said magnetic material ribbon is "a", and the width of said electrical insulating material is "b".

### BRIEF DESCRIPTION OF DRAWINGS

FIG. 1 is a schematic view showing the cross section of a magnetic core of the present invention;
FIG. 2 is a schematic view showing the cross section of a magnetic core of the prior art;
FIGS. 3 and 4 are circuit views showing an equivalent circuit of a KrF excimer laser system;
FIGS. 5 and 6 are graphs showing the temperature rise of magnetic cores wherein the ratios (W_{IN}/W_{AM}) of the width (W_{IN}) of electrical insulating materials to the width (W_{AM}) of amorphous alloys are varied;
FIG. 7 is a perspective view showing the disposition relationship between amorphous alloys and electrical insulating materials;
FIG. 8 is a graph showing the relationship between the distance C shown in FIG. 7 and the temperature rise of magnetic cores.

### BEST MODE FOR CARRYING OUT THE INVENTION

In the present invention, as shown in FIG. 1, magnetic alloy ribbons project by using the width of electrical insulating materials 2 less than the width of magnetic material ribbons 1 and the contact area of the magnetic alloy ribbons 1 to a coolant is increased. A heat removal property of heat due to heat generation of magnetic cores in use, i.e., heat generation of the magnetic material ribbons is improved.

Accordingly, in order to improve contact area of magnetic material ribbon to coolant such as air, insulating oils, fluorine-containing inert liquids, the width "b" of an electrical insulating material must be less than the width "a" of a magnetic material ribbon. If the width is too narrow, the spacing between layers becomes narrow due to the deflection occurred when the thickness of the magnetic material ribbons is thin. When a high voltage is applied, a short-circuit is liable to be generated, and therefore the width "b" of the electrical insulating material is from 0.5 "a" to less than "a" for the width "a" of the magnetic material ribbon from the standpoint of short-circuit prevention. Preferably, the width "b" of the electrical insulating material is from 0.9 "a" to less than "a". More preferably, the width "b" of the electrical insulating material is from 0.95 "a" to less than "a". The larger the ratio of the thickness of the magnetic material ribbon to the thickness of the electrical insulating material, the larger an effect due to the difference in the widths of the magnetic material ribbon and electrical insulating material.

Further, in the present invention, as shown in FIG. 1, it is preferred that both edges in a width direction of the magnetic material ribbon 1 project from both edges in a width direction of the electrical insulating material 2.

The widths of the magnetic material ribbons and the electrical insulating materials in the case of magnetic cores obtained by laminating the magnetic material ribbons and the electrical insulating materials are 1/2 of the difference in outer diameter and inner diameter of each material.

Further, the reduction of layer insulation property in ribbon edges due to the fact that the width of the electrical insulating materials is less than the width of the magnetic alloy ribbon can be compensated by insulation property of coolant for magnetic cores such as air, insulating oils and fluorine-containing inert liquids present in ribbon edges. If necessary, an insulation property is further improved by increasing the thickness of the electrical insulating materials.

The material from which the magnetic material ribbon of the present invention is produced are not particularly limited provided that the magnetic material and the electrical insulating material can be laminated or wound to form magnetic cores. Of these, iron-base amorphous alloys, cobalt-base amorphous alloys or iron-base magnetic alloys obtained by crystallizing an iron-base amorphous alloy and depositing fine grains have excellent magnetic characteristics and therefore they are preferred.

Each magnetic material described above will be described in detail. First, iron-base amorphous alloys represented by the general formula:${\text{Fe}}_{\text{100-y}} {\text{X}}_{\text{y}} \text{[at.%]}$$\text{14 ≤ y ≤ 21}$ wherein X is one or more elements selected from Si, B, P, C and Ge
have a high saturation magnetic flux density and therefore they are preferred. When X is Si or B, it is preferred that the amount of Si be from 7 to 14 at.%, and the amount of B be from 11 to 15 at.%. Of the iron-base amorphous alloys, iron-base amorphous alloys represented by the general formula:${\text{(Fe}}_{\text{1-x}} {\text{M}}_{\text{x}} {\text{)}}_{\text{100-y}} {\text{X}}_{\text{y}} \text{[at.%]}$$\text{0 < x ≤ 0.4}$$\text{14 ≤ y ≤ 21}$ wherein M is one or two elements selected from Co and Ni, and X is one or more elements selected from Si, B, P, C and Ge and wherein a portion of Fe is substituted with Co and/or Ni
are particularly preferred because high saturation magnetic flux density and high squareness ratio are obtained. In the iron-base amorphous alloys having the composition described above, magnetic characteristic can be improved by further adding not more than 5 at.% of elements such as Ti, Ta, V, Cr, Mn, Cu, Mo, Nb and W.

Further, cobalt-base amorphous alloys represented by the general formula:${\text{(Co}}_{\text{1-x}} {\text{Fe}}_{\text{x}} {\text{)}}_{\text{100-z}} {\text{(Si}}_{\text{1-y}} {\text{B}}_{\text{y}} {\text{)}}_{\text{z}}$$\text{0.02 ≤ x ≤ 0.1}$$\text{0.3 ≤ y ≤ 0.9}$$\text{20 ≤ z ≤ 30}$ have a high squareness ratio and a low core loss and therefore they are particularly preferred. In the cobalt-base amorphous alloys having the composition described above, a magnetic characteristic can be further improved by further adding not more than 8 at.% of elements such as Ti, Ta, V, Cr, Mn, Cu, Mo, Nb and W. Of these, Mn, Ni, Mo, and Nb are particularly preferred from the standpoint of a low core loss.

Preferred are the iron-base magnetic alloys obtained by crystallizing an iron-base amorphous alloy and depositing fine grains, for example, Fe-base soft magnetic alloys having the composition represented by the following general formula:${\text{(Fe}}_{\text{1-a}} {\text{M}}_{\text{a}} {\text{)}}_{\text{100-x-y-z-α-β-γ}} {\text{Cu}}_{\text{x}} {\text{Si}}_{\text{y}} {\text{B}}_{\text{z}} {\text{M}}^{\text{-}} {}_{\text{α}} {\text{M}}^{\text{--}} {}_{\text{β}} {\text{X}}_{\text{γ}}$$\text{0 ≤ a ≤ 0.5}$$\text{0.1 ≤ x ≤ 3}$$\text{0 ≤ y ≤ 30}$$\text{0 ≤ z ≤ 25}$$\text{0 ≤ y+z ≤ 35}$$\text{0.1 ≤ α ≤ 30}$$\text{0 ≤ β ≤ 10}$$\text{0 ≤ γ ≤ 10}$ wherein M is one or two elements selected from Co and Ni, and M⁻ is one or more elements selected from Nb, W, Ta, Zr, Hf, Ti and Mo, M⁻⁻ is one or more elements selected from V, Cr, Mn, Al, platinum group metals, Sc, Y, rare earth elements, Au, Zn, Sn and Re, and X is one or more elements selected from C, Ge, P, Ga, Sb, In, Be and As and wherein at least 50% of the texture is composed of fine grains, and the grains have a maximum grain size of not more than 500 Angstroms.

The amorphous alloy ribbons having the composition described above can be easily produced by applying, for example, methods such as a melt quenching method to alloys having a specific composition. Further, while the thickness of the magnetic material ribbon using these materials is not particularly limited, the thickness of the magnetic material ribbon is preferably, for example, from 3 to 40 µm and more preferably from 6 to 28 µm.

On the other hand, while the materials from which the electrical insulating material is produced are not particularly limited, polyester films are inexpensive and therefore they are preferred. Polyimide films have excellent heat-resistance and a polyimide film/magnetic material ribbon assembly can be heat treated and therefore, for example, magnetic material ribbons and polyimide films can be alternately wound or laminated and thereafter heat treated. Therefore the polyimide films are preferred. While the thickness of the electrical insulating material is not particularly limited, it is preferred that the thickness of the electrical insulating material be from 1.5 to 50 µm from the standpoint of the insulation property. More preferably, the thickness of the electrical insulating material is from 1.5 to 30 µm.

The magnetic core according to the present invention can be produced by the following process.

That is, magnetic material ribbons and electrical insulating materials having a specific composition and shape are alternately wound in a conventional method. Alternatively, the punched product obtained by punching magnetic material ribbons having a specific composition into a specific shape in a conventional method and electrical insulating materials are alternately laminated. Heat treatment is optionally applied. The magnetic characteristics such as squareness ratio of the resulting magnetic cores can be improved by heat treating in a direct-current or alternating-current magnetic field. When the cobalt-base amorphous alloys are used as the magnetic material ribbons, the composition capable of realizing a relatively high squareness ratio after melt quenching is present and therefore they can be used without applying any heat treatment.

Further, when the ribbons are heat treated in a direct-current or alternating-current magnetic field prior to the formation of magnetic cores, the squareness ratio of the resulting magnetic cores is improved as when a magnetic formed product is heat treated in a magnetic field. The size of the magnetic field is preferably of the order of 0.5 to 110 Oe and more preferably of the order of 5 to 20 Oe.

Further, combinations of the magnetic material ribbons and the electrical insulating materials can be appropriately selected depending upon required characteristics. For example, in uses wherein electrical insulating property is required, two or more layers of the electrical insulating material are used. In uses wherein magnetic characteristic is particularly required, two or more layers of the magnetic material ribbon can be used.

While the magnetic cores of the present invention are not limited provided that heat generation occurs in use in the magnetic cores wherein the magnetic material ribbons and the electrical insulating materials are alternately laminated or wound, they are particularly effective for magnetic cores used in a large electric power such as pulse generators and transformers used in lasers, particle accelerators and the like.

### EXAMPLES 1 AND 2 AND COMPARATIVE EXAMPLES 1 AND 2

Amorphous alloy ribbons and electrical insulating materials having the compositions and shapes shown in Table 1 were used and they were alternately wound to form wound magnetic cores having an outer diameter of 200 mm and an inner diameter of 100 mm. The wound magnetic cores obtained were heat treated for 30 minutes at 420°C, and thereafter heat treated for 1 hour at a constant temperature of 200°C in a direct-current constant magnetic field of 1 Oe.

### EXAMPLE 3 AND COMPARATIVE EXAMPLE 3

Amorphous alloy ribbons and electrical insulating materials having the compositions and shapes shown in Table 1 were used and they were alternately wound to form wound magnetic cores having an outer diameter of 230 mm and an inner diameter of 100 mm. The wound magnetic cores obtained were heat treated for 30 minutes at 420°C, and thereafter heat treated for 1 hour at a constant temperature of 200°C in a direct-current constant magnetic field of 1 Oe.

### EXAMPLE 4 AND COMPARATIVE EXAMPLE 4

Amorphous alloy ribbons having the compositions and shapes shown in Table 1 were alternately wound to form wound magnetic cores having an outer diameter of 200 mm and an inner diameter of 100 mm. The wound magnetic cores obtained were heat treated for 2 hours at a constant temperature of 400°C in a direct-current constant magnetic field of 1 Oe.

### EXAMPLE 5 AND COMPARATIVE EXAMPLE 5

Only amorphous alloy ribbons having the compositions and shapes shown in Table 1 were alternately wound to form wound magnetic cores having an outer diameter of 180 mm and an inner diameter of 100 mm. The amorphous alloy ribbons were heat treated for 2 hours at a constant temperature of 320°C in a direct-current constant magnetic field of 30 Oe. The amorphous alloy ribbons obtained and electrical insulating materials shown in Table 1 were used and they were alternately again wound to form wound magnetic cores having an outer diameter of 180 mm and an inner diameter of 100 mm.

### EXAMPLE 6 AND COMPARATIVE EXAMPLE 6

Amorphous alloy ribbons and electrical insulating materials having the compositions and shapes shown in Table 1 were used and they were alternately wound to form wound magnetic cores having an outer diameter of 240 mm and an inner diameter of 100 mm. The wound magnetic cores obtained were heat treated for 1 hour at a constant temperature of 550°C in a direct-current constant magnetic field of 1 Oe to crystallize amorphous alloys to deposit fine grains.

### EXAMPLE 7 AND COMPARATIVE EXAMPLE 7

Amorphous alloy ribbons having the compositions and plate thicknesses shown in Table 1 were punched into annular products having an outer diameter of 60 mm and an inner diameter of 30 mm. The annular products obtained and annular electrical insulating materials having an outer diameter of 59.5 mm and an inner diameter of 30.5 mm were alternately laminated to form laminated magnetic cores having a height of 40 mm according to Example 7.

In Comparative Example, amorphous alloy ribbons having the compositions and plate thicknesses shown in Table 1 were punched into annular products having an outer diameter of 60 mm and an inner diameter of 30 mm. The annular products obtained and annular electrical insulating materials having an outer diameter of 61 mm and an inner diameter of 29 mm were alternately laminated to form laminated magnetic cores having a height of 40 mm according to Comparative Example 7.

The magnetic cores of Examples 1, 4-6 and Comparative Examples 2, 4-6 were used in KrF excimer laser systems having an equivalent circuit of FIG. 3 whereupon the temperature rise of magnetic cores were measured. In this case, five magnetic cores were used in L_{S1} to form an oil-cooled structure. C₁₁ = 20 nF, C₂₁ = 16 nF, C₃₁ = 14 nF, and V₀ = 30 kV. The repetitive frequency is 1 kHz in Examples 1 and 3 and Comparative Examples 1 and 3, and 0.2 kHz in Examples 4, 5 and 6 and Comparative Examples 4, 5 and 6.

The results are shown in Table 1.

The magnetic cores of Examples 2 and 7 and Comparative Examples 2 and 7 were used in KrF excimer laser systems having an equivalent circuit of FIG. 4 whereupon the temperature rise of magnetic cores were measured. In this case, six magnetic cores were used in L_{S2} to form a structure cooled by a fluorine-containing inert liquid. C₁₂ = 20 nF, C₂₂ = 16 nF, V₀ = 20 kV, and repetitive frequency = 1 kHz. The results are also shown in Table 1.

As can be seen from Table 1 described hereinafter, the magnetic cores of the present invention wherein the width of the electrical insulating material is less than the width of magnetic material ribbons have small temperature rise of magnetic cores in use as compared with the prior magnetic cores wherein the width of the electrical insulating material is more than the width of the magnetic material ribbons. Even if the present magnetic cores are used as magnetic cores for high output pulse, they have an excellent cooling effect.

Further, magnetic cores were produced by varying the ratios of the width (W_{IN}) of the electrical insulating material and the width (W_{AM}) of the amorphous alloys (W_{IN}/W_{AM}), and they were used in a KrF excimer laser system having an equivalent circuit of FIG. 3. In this case, the temperature rise of the magnetic cores was measured. The results wherein the amorphous alloys and the electrical insulating materials are the same as those of Example 1 are shown in FIG. 5 and the results wherein the amorphous alloys and the electrical insulating materials are the same as those of Example 5 are shown in FIG. 6.

In this case, an oil-cooled structure was formed wherein 5 magnetic cores were in L_{S1}. C₁₁ = 20 nF, C₂₁ = 16 nF, C₃₁ = 14 nF, V₀ = 30 kV and repetitive frequency = 1 kHz.

As can be seen from FIGS. 5 and 6, the magnetic cores wherein the ratio of the width (W_{IN}) of the electrical insulating material and the width (W_{AM}) of the amorphous alloys (W_{IN}/W_{AM}) is 0.5 ≤ W_{IN}/W_{AM} < 1 have a large cooling effect and a small temperature rise and therefore they are preferred. As can be seen from FIGS. 5 and 6, FIG. 6 wherein magnetic cores comprising the amorphous alloy ribbons having a thickness of 15 µm and the electrical insulating material having a thickness of 2 µm were used i.e., magnetic cores having a large ratio of the thickness of the magnetic material ribbon to the thickness of the electrical insulating material have a large influence of the difference in width of the materials on cooling characteristic as compared with FIG. 5 wherein magnetic cores comprising the amorphous alloy ribbons having a thickness of 16 µm and the electrical insulating material having a thickness of 6 µm were used. It can be understood from FIG. 6 that, in the case of the magnetic cores having a large ratio of the thickness of the magnetic ribbons to the thickness of the electrical insulating material, the more approximate the width of the electrical insulating material is to the width of the magnetic material ribbon, the more excellent the cooling characteristic.

The reason why the temperature rise of the magnetic cores is large at W_{IN}/W_{AM} < 0.5 is thought due to heat generation by short-circuit between the amorphous alloy ribbons. Heat generation at W_{IN}/W_{AM} ≥ 1 is thought due to the reduction of heat removal property by the electrical insulating material projecting from the amorphous alloy ribbons.

In the amorphous alloys and the electrical insulating material used in Example 3, the distance C between the centerline of the amorphous alloys in a width direction and the centerline of the electrical insulating material in a width direction (see FIG. 7) was varied to prepare magnetic cores, and they were used in a KrF excimer laser system having an equivalent circuit of FIG. 3. In this case, the temperature rise of the magnetic cores was measured. The results are shown in FIG. 8.

In Examples and Comparative Examples described above, the centerline of the magnetic material ribbon and the centerline of the electrical insulating material coincide with.

In this case, an oil-cooled structure was formed wherein 5 magnetic cores were in L_{S1} of FIG. 3. C₁₁ = 20 nF, C₂₁ = 16 nF, C₃₁ = 14 nF, V₀ = 30 kV and repetitive frequency = 1 kHz.

As can be seen from FIG. 8, when the one edges of the electrical insulating material in a width direction coincides with the one edges of the magnetic material ribbon in a width direction or projects therefrom, the temperature rise of the magnetic core is increased.

Accordingly, both edges of the electrical insulating material which do not project from the magnetic material ribbon are preferred from the standpoint of the contact area of the magnetic material ribbon to a coolant.

### INDUSTRIAL APPLICABILITY

The magnetic cores of the present invention exhibit small temperature rise of the magnetic cores in use and a large cooling effect and therefore they are effective for magnetic cores used in a large electric power such as magnetic cores for high output pulse.

## Claims

1. A magnetic core, for high voltage applications, obtainable by laminating or winding a magnetic material ribbon (1) and an electrical insulating ribbon (2),
characterized in that
- said magnetic core has the relationship of 0.5a ≤ b < a in which the width of said magnetic material ribbon (1) is "a", and the width of said electrical insulating ribbon (2) is "b", the thickness of said electrical insulating ribbon (2) being sized to withstand high voltages,
- said electrical insulating ribbon (2) and said magnetic material ribbon (1) are disposed such that both edges in a width direction of the magnetic material ribbon (1) project from respective edges in a width direction of the electrical insulating ribbon (2), and wherein at least an edge of said magnetic material ribbon is capable of contacting a coolant.

2. The magnetic core according to claim 1,
wherein the relationship betwen the width "a" of said magnetic material ribbon and the width "b" of said electrical insulating ribbon has the relationship of 0.9 a ≤ b < a.

3. The magnetic core according to claim 1,
wherein the relationship between the width "a" of said magnetic material ribbon and the width "b" of said electrical insulating ribbon has the relationship of 0.95 a ≤ b < a.

4. The magnetic core according to claim 1,
wherein said magnetic material ribbon and said electrical insulating ribbon are disposed such that the centerline of the magnetic materialribbon and the centerline of said electrical insulating ribbon substantially coincide.

5. The magnetic core according to claim 1,
wherein said magnetic material ribbon is composed of an amorphous alloy represented by the following general formula:${\text{Fe}}_{\text{100-y}} {\text{X}}_{\text{y}}$$\text{14 ≤ y ≤ 21 [at.%]}$ wherein X is one or more elements selected from Si, B, P, C and Ge.

6. The magnetic core according to claim 1,
wherein said magnetic material ribbon is composed of an amorphous alloy represented by the following general formula:${\text{(Fe}}_{\text{1-x}} {\text{M}}_{\text{x}} {\text{)}}_{\text{100-y}} {\text{X}}_{\text{y}}$$\text{0 < x ≤ 0.4}$$\text{14 ≤ y ≤ 21 [at.%]}$ wherein M is one or two elements selected from Co and Ni, and X is one or more elements selected from Si, B, P, C and Ge.

7. The magnetic core according to claim 6,
wherein said magnetic material ribbon is composed of an amorphous alloy in which at least 5 at.% of one or more elements selected from Ti, Ta, V, Cr, Mn, Cu, Mo, Nb and W are further added to the amorphous alloy of claim 6.

8. The magnetic core according to claim 1,
wherein said magnetic material ribbon is composed of an amorphous alloy represented by the following general formula:${\text{(Co}}_{\text{1-x}} {\text{Fe}}_{\text{x}} {\text{)}}_{\text{100-z}} {\text{(Si}}_{\text{1-y}} {\text{B}}_{\text{y}} {\text{)}}_{\text{z}}$$\text{0.02 ≤ x ≤ 0.1}$$\text{0.3 ≤ y ≤ 0.9}$$\text{20 ≤ z ≤ 30 [at.%]}$

9. The magnetic core according to claim 8,
wherein said magnetic material ribbon is composed of an amorphous alloy in which at least 5 at.% of one or more elements selected from Ti, Ta, V, Cr, Mn, Cu, Mo, Nb and W are further added to the amorphous alloy of claim 7.

10. The magnetic core according to claim 10,
wherein said magnetic material ribbon is composed of an Fe-base soft magnetic alloy represented by the following general formula:${\text{(Fe}}_{\text{1-a}} {\text{M}}_{\text{a}} {\text{)}}_{\text{100-x-y-z-α-β-γ}} {\text{Cu}}_{\text{x}} {\text{Si}}_{\text{y}} {\text{B}}_{\text{z}} {\text{M}}^{\text{-}} {}_{\text{α}} {\text{M}}^{\text{--}} {}_{\text{β}} \text{Xγ}$$\text{0 ≤ a ≤ 0.5}$$\text{0.1 ≤ x ≤ 3}$$\text{0 ≤ y ≤ 30}$$\text{0 ≤ z ≤ 25}$$\text{0 ≤ y+z ≤ 35}$$\text{0.1 ≤ α ≤ 30}$$\text{0 ≤ β ≤ 10}$$\text{0 ≤ γ ≤ 10}$ wherein M is one or two elements selected from Co and Ni, and M⁻ is one or more elements selected from Nb, W, Ta, Zr, Hf, Ti and Mo, M⁻⁻ is one or more elements selected from V, Cr, Mn, Al, platinum group metals, Sc, Y, rare earth elements, Au, Zn, Sn and Re, and X is one or more elements selected from C, Ge, P, Ga, Sb, In, Be and As and wherein at least 50% of the texture is composed of fine grains, and the grains have a maximum grain size of not more than 50nm (500 Angstroms).

11. The magnetic core according to claim 1,
wherein said magnetic core is used in a large electric power.

12. The magnetic core according to claim 11,
wherein said magnetic core is used in pulse generators.

13. The magnetic core according to claim 11,
wherein said magnetic core is used in transformers.

## Patentansprüche

1. Magnetischer Kern für Hochspannungsanwendungen, der erhalten werden kann durch Laminieren oder Wickeln eines Bandes (1) aus magnetischem Material und eines elektrisch isolierenden Bandes (2),
dadurch **gekennzeichnet**, daß
- der magnetische Kern die Beziehung 0,5a ≤ b < a aufweist, in welcher die Breite des Bandes (1) aus magnetischem Material "a" ist, und die Breite des elektrisch isolierenden Bandes (2) "b" ist, wobei die Dicke des elektrisch isolierenden Bandes (2) bemessen ist, Hochspannungen zu widerstehen,
- das elektrisch isolierende Band (2) und das Band (1) aus magnetischem Material so angeordnet sind, daß beide Kanten des Bandes (1) aus magnetischem Material in einer Breitenrichtung von jeweiligen Kanten in einer Breitenrichtung des elektrisch isolierenden Bandes (2) vorstehen, und worin wenigstens eine Kante des Bandes aus magnetischem Material in der Lage ist, ein Kühlmittel zu kontaktieren.

2. Magnetischer Kern nach Anspruch 1, dadurch gekennzeichnet, daß die Beziehung zwischen der Breite "a" des Bandes aus magnetischem Material und der Breite "b" des elektrisch isolierenden Bandes die Beziehung 0,9a ≤ b < a aufweist.

3. Magnetischer Kern nach Anspruch 1, dadurch gekennzeichnet, daß die Beziehung zwischen der Breite "a" des Bandes aus magnetischem Material und der Breite "b" des elektrisch isolierenden Bandes die Beziehung 0,95a ≤ b < a aufweist.

4. Magnetischer Kern nach Anspruch 1, dadurch gekennzeichnet, daß das Band aus magnetischem Material und das elektrisch isolierende Band so angeordnet sind, daß die Mittellinie des Bandes aus magnetischem Material und die Mittellinie des elektrisch isolierenden Bandes im wesentlichen zusammenfallen.

5. Magnetischer Kern nach Anspruch 1, dadurch gekennzeichnet, daß das Band aus magnetischem Material aus einer amorphen Legierung gebildet ist, die durch die folgende allgemeine Formel dargestellt wird:${\text{Fe}}_{\text{100-y}} {\text{X}}_{\text{y}}$$\text{14 ≤ y ≤ 21 [at.%]}$ worin X ein oder mehrere Elemente ist, die gewählt sind von Si, B, P, C und Ge.

6. Magnetischer Kern nach Anspruch 1, dadurch gekennzeichnet, daß das Band aus magnetischem Material aus einer amorphen Legierung gebildet ist, die durch die folgende allgemeine Formel dargestellt wird:${\text{(Fe}}_{\text{1-x}} {\text{M}}_{\text{x}} {\text{)}}_{\text{100-y}} {\text{X}}_{\text{y}}$$\text{0 < x ≤ 0.4}$$\text{14 ≤ y ≤ 21 [at.%]}$ worin M ein oder zwei Elemente ist, die gewählt sind von Co und Ni, und X ein oder mehrere Elemente ist, die gewählt sind von Si, B, P, C und Ge.

7. Magnetischer Kern nach Anspruch 6, dadurch gekennzeichnet, daß das Band aus magnetischem Material aus einer amorphen Legierung gebildet ist, in welcher wenigstens 5 Atom-% von einem oder mehreren Elementen, die gewählt sind von Ti, Ta, V, Cr, Mn, Cu, Mo, Nb und W, der amorphen Legierung nach Anspruch 6 hinzugefügt sind.

8. Magnetischer Kern nach Anspruch 1, dadurch gekennzeichnet, daß das Band aus magnetischem Material aus einer amorphen Legierung gebildet ist, die durch die folgende allgemeine Formel dargestellt wird:${\text{(Co}}_{\text{1-x}} {\text{Fe}}_{\text{x}} {\text{)}}_{\text{100-z}} {\text{(Si}}_{\text{1-y}} {\text{B}}_{\text{y}} {\text{)}}_{\text{z}}$$\text{0.02 ≤ x ≤ 0.1}$$\text{0.3 ≤ y ≤ 0.9}$$\text{20 ≤ z ≤ 30 [at.%]}$

9. Magnetischer Kern nach Anspruch 8, dadurch gekennzeichnet, daß das Band aus magnetischem Material aus einer amorphen Legierung gebildet ist, in welcher wenigstens 5 Atom-% von einem oder mehreren Elementen, die von Ti, Ta, V, Cr, Mn, Cu, Mo, Nb und W gewählt sind, der amorphen Legierung nach Anspruch 7 hinzugefügt sind.

10. Magnetischer Kern nach Anspruch 10, dadurch gekennzeichnet, daß das Band aus magnetischem Material aus einer Fe-basierenden, weichmagnetischen Legierung gebildet ist, die durch die folgende allgemeine Formel dargestellt wird:${\text{(Fe}}_{\text{1-a}} {\text{M}}_{\text{a}} {\text{)}}_{\text{100-x-y-z-α-β-γ}} {\text{Cu}}_{\text{x}} {\text{Si}}_{\text{y}} {\text{B}}_{\text{z}} {\text{M}}^{\text{-}} {}_{\text{α}} {\text{M}}^{\text{--}} {}_{\text{β}} {\text{X}}_{\text{γ}}$$\text{0 ≤ a ≤ 0.5}$$\text{0.1 ≤ x ≤ 3}$$\text{0 ≤ y ≤ 30}$$\text{0 ≤ z ≤ 25}$$\text{0 ≤ y+z ≤ 35}$$\text{0.1 ≤ α ≤ 30}$$\text{0 ≤ β ≤ 10}$$\text{0 ≤ γ ≤ 10}$ worin M eines oder zwei Elemente ist, die gewählt sind von Co und Ni, und M⁻ ein oder mehrere Elemente ist, die gewählt sind von Nb, W, Ta, Zr, Hf, Ti und Mo, M⁻⁻ ein oder mehrere Elemente ist, die gewählt sind von V, Cr, Mn, Al, Metallen der Platingruppe, Sc, Y, Elementen der seltenen Erden, Au, Zn, Sn und Re, und X ein oder mehrere Elemente ist, die gewählt sind von C, Ge, P, Ga, Sb, In, Be und As, und worin wenigstens 50% der Struktur aus feinen Körnern gebildet ist, und die Körner eine maximale Korngröße von nicht mehr als 50 nm (500 Angström) haben.

11. Magnetischer Kern nach Anspruch 1, dadurch gekennzeichnet, daß der magnetische Kern in einer Hochleistungsanwendung eingesetzt ist.

12. Magnetischer Kern nach Anspruch 11, dadurch gekennzeichnet, daß der Magnetischen Kern in Impulsgeneratoren verwendet wird.

13. Magnetischer Kern nach Anspruch 11, dadurch gekennzeichnet, daß der magnetische Kern in Transformatoren verwendet wird.

## Revendications

1. Noyau magnétique pour des applications haute tension, pouvant être obtenu en stratifiant ou en bobinant un ruban (1) de matériau magnétique et un ruban (2) électriquement isolant, caractérisé en ce que
- ledit noyau magnétique présente la relation 0,5a ≤ b < a, dans laquelle "a" représente la largeur dudit ruban (1) de matériau magnétique et "b" représente la largeur dudit ruban (2) électriquement isolant, l'épaisseur dudit ruban électriquement isolant (2) étant dimensionnée pour supporter de hautes tensions,
- ledit ruban électriquement isolant (2) et ledit ruban (1) de matériau magnétique sont disposés de telle sorte que les deux bords dans la direction d'une largeur du ruban (1) de matériau magnétique débordent par rapport aux bords respectifs, dans la direction d'une largeur du ruban (2) électriquement isolant, et dans lequel au moins un bord dudit ruban de matériau magnétique est capable d'entrer en contact avec un agent de refroidissement.

2. Noyau magnétique selon la revendication 1, dans lequel la relation entre la largeur "a" dudit ruban de matériau magnétique et la largeur "b" dudit ruban électriquement isolant est la relation 0,9 a ≤ b < a.

3. Noyau magnétique selon la revendication 1, dans lequel la relation entre la largeur "a" dudit ruban de matériau magnétique et la largeur "b" dudit ruban électriquement isolant est la relation 0,95 a ≤ b < a.

4. Noyau magnétique selon la revendication 1, dans lequel ledit ruban de matériau magnétique et ledit ruban électriquement isolant sont disposés de telle sorte que l'axe du ruban de matériau magnétique et l'axe dudit matériau électriquement isolant coïncident essentiellement.

5. Noyau magnétique selon la revendication 1, dans lequel ledit ruban de matériau magnétique est composé d'un alliage amorphe représenté par la formule générale ci-dessous:${\text{Fe}}_{\text{100-y}} {\text{X}}_{\text{y}}$$\text{14 ≤ y ≤ 21 [% atomiques]}$ dans laquelle X représente un ou plusieurs éléments choisis parmi Si, B, P, C et Ge.

6. Noyau magnétique selon la revendication 1, dans lequel ledit ruban de matériau magnétique est composé d'un alliage amorphe représenté par la formule générale ci-dessous:${\text{(Fe}}_{\text{1-x}} {\text{M}}_{\text{x}} {\text{)}}_{\text{100-y}} {\text{X}}_{\text{y}}$$\text{0 < x ≤ 0,4}$$\text{14 ≤ y ≤ 21 [% atomiques]}$ dans laquelle M représente un ou deux éléments choisis parmi Co et Ni, et X représente un ou plusieurs éléments choisis parmi Si, B, P, C et Ge.

7. Noyau magnétique selon la revendication 6, dans lequel ledit ruban de matériau magnétique est composé d'un alliage amorphe dans lequel au moins 5% atomiques d'un ou plusieurs éléments choisis parmi Ti, Ta, V, Cr, Mn, Cu, Mo, Nb et W sont en outre ajoutés à l'alliage amorphe de la revendication 6.

8. Noyau magnétique selon la revendication 1, dans lequel ledit ruban de matériau magnétique est composé d'un alliage amorphe représenté par la formule générale:${\text{(Co}}_{\text{1-x}} {\text{Fe}}_{\text{x}} {\text{)}}_{\text{100-z}} {\text{(Si}}_{\text{1-y}} {\text{B}}_{\text{y}} {\text{)}}_{\text{z}}$$\text{0,02 ≤ x ≤ 0,1}$$\text{0,3 ≤ y ≤ 0,9}$$\text{20 ≤ z ≤ 30 [% atomiques]}$

9. Noyau magnétique selon la revendication 8, dans lequel ledit ruban de matériau magnétique est composé d'un alliage amorphe dans lequel au moins 5% atomiques d'un ou plusieurs éléments choisis parmi Ti, Ta, V, Cr, Mn, Cu, Mo, Nb et W sont en outre ajoutés à l'alliage amorphe de la revendication 7.

10. Noyau magnétique selon la revendication 10, dans lequel ledit ruban de matériau magnétique est composé d'un alliage magnétique doux à base de Fe, représenté par la formule générale ci-dessous:${\text{(Fe}}_{\text{1-a}} {\text{M}}_{\text{a}} {\text{)}}_{\text{100-x-y-z-α-β-γ}} {\text{Cu}}_{\text{x}} {\text{Si}}_{\text{y}} {\text{B}}_{\text{z}} {\text{M}}^{\text{-}} {}_{\text{α}} {\text{M}}^{\text{--}} {}_{\text{β}} {\text{X}}_{\text{γ}}$$\text{0 ≤ a ≤ 0,5}$$\text{0,1 ≤ x ≤ 3}$$\text{0 ≤ y ≤ 30}$$\text{0 ≤ z ≤ 25}$$\text{0 ≤ y+z ≤ 35}$$\text{0,1 ≤ α ≤ 30}$$\text{0 ≤ β ≤ 10}$$\text{0 ≤ γ ≤ 10}$ dans laquelle M représente un ou deux éléments choisis parmi Co et Ni, et M⁻ représente un ou plusieurs éléments choisis parmi Nb, W, Ta, Zr, Hf, Ti et Mo, M⁻⁻ représente un ou plusieurs éléments choisis parmi V, Cr, Mn, Al, des métaux du groupe du platine, Sc, Y, des éléments des terres rares, Au, Zn, Sn et Re, et X représente un ou plusieurs éléments choisis parmi C, Ge, P, Ga, Sb, In, Be et As, et dans lequel au moins 50% de la texture est composée de grains fins, et les grains présentent une taille de grain maximale qui n'est pas supérieure à 50 nm (500 Angstroems).

11. Noyau magnétique selon la revendication 1, dans lequel ledit noyau magnétique est utilisé à une puissance électrique élevée.

12. Noyau magnétique selon la revendication 11, dans lequel ledit noyau magnétique est utilisé dans des générateurs d'impulsions.

13. Noyau magnétique selon la revendication 11, dans lequel ledit noyau magnétique est utilisé dans des transformateurs.
